

## UNITED STATES PATENT OFFICE

2,250,929

MANUFACTURE OF IMPROVED FILAMENTS,  
THREADS, FOILS, OR SHEETS OF CELLULOSE ESTERS OR ETHERSJohn Gwynant Evans and Arnold Shepherdson,  
Manchester, England, assignors to Imperial  
Chemical Industries Limited, a corporation of  
Great BritainNo Drawing. Application March 28, 1938, Serial  
No. 198,583. In Great Britain March 31, 1937

13 Claims. (Cl. 18—54)

This invention relates to the manufacture of improved filaments, threads, foils or sheets of cellulose esters or ethers.

In the manufacture of filaments, threads, foils or sheets of cellulose esters or ethers it is customary to extrude a spinning solution, which comprises a solution of the said esters or ethers in suitable organic solvents together with suitable softeners, plasticisers, or other ingredients as necessary, through a suitably shaped orifice so that the solvents are volatilised from the extruded mass as in the dry spinning process, or so that the extruded mass is coagulated in a coagulating bath, as in the wet spinning process. The drying atmosphere in the former case and the coagulating bath in the latter case may both be regarded as setting media for the extruded mass. The extruded mass may or may not be subjected to tension whilst it is still in a plastic condition.

For convenience, the filaments, threads, foils or sheets thus produced will hereinafter be referred to generically as cellulosic shaped material, bearing in mind that the cross-section of the resulting filament, thread, foil or sheet etc. is determined and shaped by the outline of the orifice employed and subsequent tension treatment where employed.

According to the present invention we incorporate into the spinning solutions of the kind referred to a quaternary ammonium salt as hereinafter defined and, having formed filaments, threads, foils or sheets by wet or dry spinning in the customary manner, we subject the said filaments, threads, foils or films to a heat treatment at temperatures above 70° C.

The quaternary ammonium salts to be used according to the present invention are compounds of the general formula:  $R-X-CH_2-N(tert)-Y$ , wherein R is a long-chain aliphatic radical, having not less than 12 carbon atoms, it may, however, be a saturated or unsaturated hydrocarbon radical; also, it may be the radical of a long chain carboxylic acid, i. e. of what is commonly known as a fatty acid in the original etymological sense, that is, it may have the form  $R'-CO$ , wherein R' is an aliphatic hydrocarbon radical of not less than 11 carbon atoms; X is a carbon-to-carbon linking member and may be oxygen, sulphur, or an imino or substituted imino group. Among the substituted imino groups may be mentioned alkylimino, such as methylimino or ethylimino; acylamido, such as acetamido, aralkylimino, such as benzylimino; arylimino, such as anilino; and finally, the residue

of a carbamate, for instance, the residue of methyl carbamate,



or ethylcarbamate



10 the group N(tert) may represent the residue of a tertiary aliphatic base, or may stand for the residue of a heterocyclic base, such as pyridine or quinoline; finally, the symbol Y stands for the monovalent anion of an acid, for instance, of hydrochloric, hydrobromic, nitric, sulphuric, p-toluenesulphonic, oxalic, and the like.

15 Suitable quaternary salts may be made, for example, by the methods described in British specifications Nos. 390,553, 394,196, 471,130, 475,119, 475,170.

20 As quaternary ammonium salts suitable to be used in the process of the invention there may be mentioned, for example, octadecyloxymethylpyridinium chloride, octadecyloxymethylpyridinium bromide, octadecyloxymethylpyridinium iodide, octadecyloxymethylpyridinium nitrate, octadecyloxymethylpyridinium acid oxalate, 25 octadecyloxymethylpyridinium pyridine sulphite, cetylthiomethyl pyridinium bromide, octadecyloxymethyltriethylammonium chloride, octadecyloxymethyltriethanolammonium chloride, octadecyloxymethylquinolinium chloride; pyridinium derivatives from the chloromethyl ethers of sperm oil alcohols, lauramidomethylpyridinium 30 chloride, stearamidomethylpyridinium chloride, stearamidomethylpyridinium bromide, stearamidomethylpyridinium nitrate, stearamidomethylpyridinium pyridine sulphite, stearamidomethylpyridinium m-nitrobenzene sulphonate, N-40 methyl-stearamidomethylpyridinium chloride, stearanilidomethylpyridinium chloride; oleylamidomethylpyridinium chloride, N-carbomethoxyheptadecylaminomethylpyridinium chloride, p-cetylphenylaminomethylpyridinium pyridine sulphite, and p-stearamidophenylaminomethylpyridinium pyridine sulphite.

45 The defined quaternary ammonium salts are soluble in many of the solvents commonly used for the making up of spinning solutions such as, for example, acetone, mixtures of acetone and methyl formate, methyl or ethyl acetates, acetylacetone or diacetone alcohol. Thus the quaternary salts may conveniently be incorporated by dissolving in the already made spinning solution or, preferably, by dissolving the salts in

a suitable solvent and admixing with the already made spinning solution or with one or more of the ingredients thereof before making up the spinning solution. The quaternary salts may be incorporated if desired in the form of suspensions or dispersions in a suitable liquid medium provided that the solid particles in the said suspensions or dispersions are not so large that they block or foul the spinning orifice.

Filaments, threads, foils or sheets made in accordance with the present invention are characterised by their water-repellent properties. Further, the filaments, threads or woven fabrics made therefrom have a remarkable softness of handle. The water-repellent properties and soft handle are resistant to laundering and dry-cleaning.

The invention is illustrated but not limited by the following examples, in which the parts are by weight.

*Example 1*

To 1000 parts of a 25% solution of cellulose acetate in a mixture of 950 parts of acetone and 50 parts of water, there is added 1000 parts of acetone containing 5 parts of stearamidomethylpyridinium bromide (which may be prepared by reacting pyridine with stearamidomethyl bromide; see British specification No. 471,130). The resulting spinning solution is forced through a spinning nozzle into a current of warm air in the known manner. The filaments so formed are, when dry, subjected to a dry heat for 10 minutes at 120° C. The resultant filaments have water-repellent properties which are resistant to washing and dry cleaning treatments.

*Example 2*

To a solution of 200 parts of commercial cellulose acetate in 800 parts of a mixture of acetone and water (96% acetone, 4 parts water), there are added 4 parts of octadecyloxymethylpyridinium chloride dissolved in 46 parts of ethanol. This solution is extruded through spinning dies in the usual manner into a warm atmosphere of acetone vapour and the threads thus formed are freed from solvent by drying in a current of warm air.

The dried threads are now heated for 2½ minutes at 150° C. The threads so obtained are water-repellent and are softer than threads similarly spun from solutions containing no octadecyloxymethylpyridinium chloride. The water-repellent properties are resistant to washing and to dry-cleaning treatments.

*Example 3*

To a solution containing 150 parts of commercial cellulose acetate dissolved in 850 parts of a mixture of acetone and water (95% acetone, 5% water), there are added 3 parts of the mixed pyridinium chlorides derived from the chloromethyl ethers of sperm oil alcohols contained in 47 parts of acetone.

This solution is extruded and the threads are dried and heated as described in Example 2. After the heat treatment the threads are immersed for a few minutes at 45° in a solution of 1 part of soap and 1 part of ammonia (sp. gr. 0.88) in 1000 parts of water. The threads are well rinsed and dried.

The threads thus produced are highly water-repellent and very much softer than threads formed in the absence of the quaternary salts. Fabrics woven from these threads are remarkable for the ease with which they fall into pleas-

ing folds. These properties are resistant to washing and dry-cleaning treatments.

*Example 4*

5 To 50 parts of commercial cellulose acetate dissolved in 900 parts of acetone there are added 2 parts of stearamidomethylpyridinium nitrate dissolved in 48 parts of warm ethanol. This solution is extruded into a 23% aqueous solution of calcium chloride and the threads thus formed are dried rapidly at 50°-60° C. in a current of warm air. The dry threads are then heated at 120° C. for 10 minutes.

10 After the heat treatment the threads are immersed for a few minutes at 40° C. in a solution containing 0.5 part of oleyl sodium sulphate and 1 part of ammonia per 1000 parts of water. The threads are well rinsed and dried.

15 Threads thus treated are water-repellent and very much softer than threads formed in the absence of the stearamidomethylpyridinium nitrate.

These properties are resistant to washing and dry-cleaning processes.

20 25 In the above example suitable additions may be made to the spinning solution or to the coagulating bath to assist in the production of uniform homogeneous fibres. For instance, benzene and alcohol or pyridine or aniline may be added to the spinning solution, or the coagulating solution may contain thiocyanates or water soluble solvents or swelling agents for cellulose acetate, such as acetone, diacetone alcohol or ethanol.

*Example 5*

To 100 parts of cellulose formate (formyl content 20%) dissolved in 900 parts of acetone there are added 3 parts of octadecyloxymethylquinolinium bromide dissolved in 47 parts of ethanol. The solution is extruded into a 23% solution of calcium chloride and the threads thus formed are dried rapidly in a current of warm air at 40°-50° C.

45 The dry threads are heated for 10 minutes at 125° C. and are then washed as described in the preceding example.

50 The threads produced are highly water-repellent and considerably softer than threads of cellulose formate, made in the absence of octadecyloxymethylquinolinium bromide. These properties are resistant to washing and to dry-cleaning treatments.

*Example 6*

55 To 50 parts of acetone soluble ethyl cellulose dissolved in 950 parts of acetone there are added 1 part of cetylloxymethylpyridinium pyridine sulphite and 0.1 part of hexamethylene tetramine dissolved in 49 parts of ethanol. This solution is extruded into an atmosphere of acetone vapour at a temperature of 40-50° C.

60 The threads of ethyl cellulose thus formed are freed from acetone by drying in a current of warm air and are then heated for 2½ minutes at 150° C. The threads are then washed for a few minutes at 40° C. in a solution containing 1 part of soap and 1 part of ammonia in 1000 parts of water and then well rinsed and dried.

65 70 The threads thus formed are highly water-repellent and softer than threads formed in the absence of cetylloxymethylpyridinium pyridine sulphite.

These properties are resistant to washing and dry cleaning treatments.

We claim:

1. The process of imparting water-repellency and softness characteristics to cellulosic shaped material of the class formed by extrusion molding from cellulosic raw material of the group consisting of cellulose esters and cellulose ethers, which comprises incorporating into a solution of said raw material, in an organic solvent, a quaternary ammonium compound of the general formula  $R-X-CH_2-N(tert)-Y$ , wherein  $R$  is a long-chain aliphatic radical selected from the group consisting of aliphatic hydrocarbon radicals and aliphatic hydrocarbon acyl radicals having not less than 12 carbon atoms,  $X$  is a carbon-to-carbon linking member selected from the group consisting of oxygen, sulfur and the imino radicals,  $N(tert)$  represents the molecule of a tertiary organic base, while  $Y$  is the anion of a water-soluble acid; then subjecting said solution to extrusion and setting to form shaped material, and finally subjecting said formed material to heat treatment in the absence of moisture at a temperature not less than 70° C.

2. The process of imparting water-repellency and softness characteristics to cellulosic shaped material of the class formed by extrusion molding from cellulosic raw material of the group consisting of cellulose esters and cellulose ethers, which comprises incorporating into a solution of said raw material, in an organic solvent, a quaternary ammonium compound of the general formula  $R-CONH-CH_2-N(tert)-Y$ , wherein  $R$  is a long-chain aliphatic hydrocarbon radical having not less than 11 carbon atoms,  $N(tert)$  represents the molecule of a tertiary organic base, while  $Y$  is the anion of a water-soluble acid; then subjecting said solution to extrusion and setting to form shaped material, and finally subjecting said formed material to heat treatment in the absence of moisture at a temperature not less than 70° C.

3. The process of imparting water-repellency and softness characteristics to cellulosic shaped material of the class formed by extrusion molding from cellulosic raw material of the group consisting of cellulose esters and cellulose ethers, which comprises incorporating into a solution of said raw material, in an organic solvent, a quaternary ammonium compound of the general formula



wherein  $R'$  is a lower alkyl radical,  $R$  is a long-chain aliphatic hydrocarbon radical having not less than 12 carbon atoms,  $N(tert)$  represents the molecule of a tertiary organic base, while  $Y$  is the anion of a water-soluble acid; then subjecting said solution to extrusion and setting to form shaped material, and finally subjecting said formed material to heat treatment in the absence of moisture at a temperature not less than 70° C.

4. The process of imparting water-repellency and softness characteristics to cellulosic shaped material of the class formed by extrusion molding from cellulosic raw material of the group consisting of cellulose esters and cellulose ethers, which comprises incorporating into a solution of said raw material, in an organic solvent, a quaternary ammonium compound of the general formula  $R-O-CH_2-N(tert)-Y$ , wherein  $R$  is a long-chain aliphatic hydrocarbon radical having not less than 12 carbon atoms,  $N(tert)$  represents the molecule of a tertiary organic base,

5 while  $Y$  is the anion of a water-soluble acid; then subjecting said solution to extrusion and setting to form shaped material, and finally subjecting said formed material to heat treatment in the absence of moisture at a temperature not less than 70° C.

6. The process of imparting water-repellency and softness characteristics to cellulosic shaped material of the class formed by extrusion molding from cellulosic raw material of the group consisting of cellulose esters and cellulose ethers, which comprises incorporating into a solution of said raw material, in an organic solvent, a quaternary ammonium compound of the general formula



20 where R is a long-chain aliphatic hydrocarbon radical having not less than 11 carbon atoms, 25 while Y is the anion of a water-soluble acid; then subjecting said solution to extrusion and setting to form shaped material, and finally subjecting said formed material to heat treatment in the absence of moisture at a temperature not less than 70° C.

30 6. The process of imparting water-repellency and softness characteristics to cellulosic shaped material of the class formed by extrusion molding from cellulosic raw material of the group consisting of cellulose esters and cellulose ethers, which comprises incorporating into a solution of said raw material, in an organic solvent, a quaternary ammonium compound of the general formula



45 where R is a long-chain aliphatic hydrocarbon radical having not less than 12 carbon atoms, 50 while Y is the anion of a water-soluble acid; then subjecting said solution to extrusion and setting to form shaped material, and finally subjecting said formed material to heat treatment in the absence of moisture at a temperature not less than 70° C.

60 7. The process of improving the feel and water-repellency characteristics of cellulose acetate textile material, which comprises forming a solution of cellulose acetate in acetone, incorporating into said solution further a stearamido-methyl pyridinium salt of a water-soluble acid, then subjecting the solution to extrusion and setting to form a shaped textile material, and finally subjecting said textile material to heat treatment in the absence of moisture at a temperature between 120 and 150° C.

65 8. Artificial cellulosic material of the group consisting of filaments, threads, foils and sheets of cellulose esters and of cellulose ethers, characterized by having a water-repellent surface, said material having incorporated within its body the reaction product obtainable by heating in contact with said cellulosic material but in the absence of moisture and at a temperature

between 120 and 150° C., a quaternary ammonium compound of the general formula



wherein R is a long-chain aliphatic radical selected from the group consisting of aliphatic hydrocarbon radicals and aliphatic hydrocarbon acyl radicals having not less than 12 carbon atoms, X is a carbon-to-carbon linking member selected from the group consisting of oxygen, sulfur and the imino radicals, N(tert) represents the molecule of a tertiary organic base, while Y is the anion of a water-soluble acid.

9. Artificial cellulosic shaped material characterized by having a soft feel and a water-repellent surface, said material being the product of a process as defined in claim 6.

10. Artificial cellulosic shaped material characterized by having a soft feel and a water-repellent surface, said material being the product of a process as defined in claim 7.

11. Artificial cellulosic shaped material characterized by having a soft feel and a water-repellent surface, said material being the product of a process as defined in claim 8.

12. Artificial cellulosic textile material of the group consisting of cellulose esters and cellulose

ethers, characterized by having a soft feel and a water-repellent surface, said material having incorporated within its fiber the reaction product obtainable by heating stearamido-methyl-pyridinium chloride, in contact with said cellulosic material but in the absence of moisture at a temperature between 120 and 150° C.

13. A water-repellent cellulosic shaped material of the class formed by extrusion molding 10 from an organic solution of a compound of the group consisting of cellulose esters and of cellulose ethers, said material including within its structure a substantially homogeneous combination of the said cellulosic material with a water-repellency agent of the group having the general formula R-X-CH<sub>2</sub>-N(tert)-Y, wherein R is a long-chain aliphatic radical selected from the group consisting of aliphatic hydrocarbon radicals and aliphatic hydrocarbon acyl radicals having not less than 12 carbon atoms, X is a carbon-to-carbon linking member selected from the group consisting of oxygen, sulfur and the imino radicals, N(tert) represents the molecule of a tertiary organic base, while Y is the anion of a water-soluble acid.

JOHN GWYNANT EVANS.  
ARNOLD SHEPHERDSON.